# EUROPEAN PATENT SPECIFICATION

(11) **EP 0 218 160 B1**
(45) Date of publication and mention of the grant of the patent: **06.12.1989**
(21) Application number: 86113306.4
(22) Date of filing: 26.09.1986
(51) Int. Cl.: B41N 1/08, C25D 11/24

(54) **Treated anodized aluminum support and lithographic printing plate containing same**
Behandelter Träger aus anodisiertem Aluminium und den Täger enthaltende lithographische Druckplatte
Support en aluminium anodisé soumis à un traitement et plaque d'impression lithographique le comprenant

(30) Priority: 10.10.1985 US 786403
(43) Date of publication of application: 15.04.1987
(73) Proprietor: EASTMAN KODAK COMPANY (a New Jersey corporation), Rochester, New York 14650 (US)
(72) Inventor: Gilson, Richard E., Rochester New York 14650 (US); Miller, Gary R., Windsor Colorado 80551 (US)
(74) Representative: Parent, Yves

(56) References cited:
- DE-A- 1 571 890
- FR-A- 2 211 675
- FR-A- 2 385 819

## Description

This invention relates to a support material for use in a lithographic printing plate, to a method for the preparation of the support material, and to a lithographic printing plate comprising such support material which exhibits improved press sensitivity and extended shelf-life.

One important characteristic of any presensitized lithographic printing plate is the ability to remain stable and yield reproducible photographic speed performance between the time the plate is manufactured and subsequently used. Yet another important property is the ability of the plate to shed ink from non-image areas during start-up and throughout the useful life of the plate.

U.S. patent 4,492,616 describes a process for treating aluminum oxide layers by treating the metal surface with an aqueous alkali metal silicate solution and an aqueous solution containing alkaline earth metal ions.

U.S. patent 3,860,426 describes a lithographic printing plate having a hydrophilic cellulosic subbing layer containing a water-soluble salt of a metal to reduce scumming of the plate in areas in which the printing layer is removed. While these plates have gained widespread commercial acceptance, they have not been found to yield reproducible speed performance between the time the plate is manufactured and used under all storage and handling conditions encountered. Moreover, the printing industry has demanded more stringent requirements regarding press sensitivity in their efforts to minimize variability and waste.

Thus, there is a need for lithographic printing plates exhibiting improved press sensitivity and extended shelf-life.

In accordance with the present invention there is provided a lithographic printing plate exhibiting improved press sensitivity and extended shelf-life.

The invention provides a lithographic printing plate support material comprising an anodized aluminum plate having an anodic layer, a silicate layer in contact with the anodic layer, and a metal salt layer, in contact with the silicate layer, which comprises a metal salt having the formula MX, wherein M is a metal selected from the group consisting of zinc, magnesium, nickel and chromium and X is an anion selected from the group consisting of acetate, chloride and borate.

The invention further provides a method for preparing a lithographic printing plate support material comprising the steps of a) contacting an anodized aluminum plate with a silicate and b) contacting the silicated plate with a metal salt having the formula MX, wherein M is a metal selected from the group consisting of zinc, magnesium, nickel and chromium and X is an anion selected from the group consisting of acetate, chloride and borate.

A lithographic printing plate in accordance with the present invention comprises a) a lithographic printing plate support material comprising an anodized aluminum plate having an anodic layer, a silicate layer in contact with the anodic layer, and a metal salt layer, in contact with the silicate layer which comprises a metal salt having the formula MX wherein M is a metal selected from the group consisting of zinc, magnesium, nickel, and chromium and X is an anion selected from the group consisting of acetate, chloride, and borate, and b) a radiation sensitive layer. The lithographic printing plate of this invention exhibits improved press sensitivity and extended shelf-life.

The support material comprises an aluminum or aluminum alloy plate. Suitable aluminum alloys are alloys with sinc, silicon, chromium, copper, manganese, magnesium, chromium, zinc, lead, bismuth, nickel, iron or titanium which may contain negligible amounts of impurities.

The surface of the aluminum plate is preferably subjected to chemical cleaning such as degreasing with solvents or alkaline agents for the purpose of exposing a clean surface free of grease, rust or dust which is usually present on the aluminum surface. Preferably, the surface is grained. Suitable graining methods include glass bead graining, ball graining, sand blasting, brush graining and electrolytic graining. Following the graining operation, the support can be treated with an aluminum etching agent and a desmutting acid bath.

An anodized stratum is then formed on the aluminum plate. This stratum is referred to herein as an anodic layer. An electric current is passed through the support immersed as a cathode in a solution containing one or more acids selected from phosphoric acid, sulfuric acid, oxalic acid, boric acid, chromic acid, sulfamic acid, and benzene-sulfonic acid. An anodized stratum is thus formed on the surface of the support.

After anodizing, the surface of the anodized aluminum plate is contacted with a silicating agent such as an alkali metal silicate, salcium silicate, silicic acid, colloidal silica or polymerized silicic acid to silicate the plate. The silicate treatment renders the anodized surface hydrophilic. Preferably, the support is treated with an aqueous solution of the silicating agent. The silicating agent preferably is present at a concentration of about 0.5 to about 10% and the temperature of the solution preferably is 20°C to 100°C, most preferably 60°C to 100°C. The optimum dwell time of the plate in the solution depends on the solution temperature, the silicating agent concentration and the ultimate intended use of the lithographic plate. A dwell time of 15 to 80 seconds has been found to be particularly advantageous.

After the plate is silicated, the silicated plate is contacted with a metal salt having the formula MX wherein M is a metal selected from the group consisting of zinc, magnesium, nickel, and chromium and X is an anion selected from the group consisting of acetate, chloride, and borate. A thin treatment or layer, probably often substantially of monomolecular thickness of the metal salt is thus provided. Metal salt molecules are deposited upon the surface uniformly or non-uniformly, provided that the layer is present in a coverage from 10 to 50 mg/m², preferably from 20 to 40 mg/m². The metal salts which are particularly useful include water soluble salts of zinc, magnesium, nickel, and chromium,. The salts are formed by methods known in the art. Useful salts include acetate, chloride, and borate. The support preferably is immersed in an aqueous bath containing the metal salt at a concentration of from 0.1 % to 45%, the higher concentration being limited only by the solubility of the metal salt. A preferred metal salt bath concentration is 1% to 10%, most preferably 2% to 5%. The metal salt layer can consist essentially of the above-described metal salt. The bath can be operated from room temperature to boiling; however, a temperature of 30°C-80°C is preferable. Excellent results have been achieved with a bath temperature of 50°C-70°C. The dwell time of the plate in the bath depends on concentration and temperature. A dwell time of 10 seconds to 5 minutes has been found acceptable under many conditions. Preferably, the dwell time is 15 seconds to 3 minutes such that the treatment is conducive to a continuous process.

The lithographic printing plate support material of this invention can be coated, if desired, with a thin coating of a hydrophilic material which serves as a subbing layer. The hydrophilic coating contributes to improving the water receptivity of the non-printing areas of the processed plate. Preferably, the hydrophilic coating is coated over a support treated as described above. The hydrophilic coating is coated by known techniques in a subbing amount. It is particularly advantageous to use a water-soluble permanently hydrophilic material which can be coated from an aqueous dispersion. A solution containing polyacrylamide is especialy advantageous for this purpose, as are solutions containing carboxymethyl cellulose, polyvinylphosphonic acid, sodium silicate and combinations of these. Other polymers useful in forming hydrophilic interlayers include polyvinylalcohol, copolymers of maleic anhydride with ethylene, vinyl acetate, styrene or vinyl methyl ether, polyacrylic acid, hydroxymethyl cellulose and polyvinyl pyrrolidone.

The lithographic printing plate in accordance with this invention comprises a) a lithographic printing plate support material comprising an anodized aluminum plate having an anodic layer, a silicate layer in contact with the anodic layer, and a metal salt layer, in contact with the silicate layer, which comprises a metal salt having the formula MX wherein M is a metal selected from the group consisting of zinc, magnesium, nickel, and chromium and X is an anion selected from the group consisting of acetate, chloride, and borate, and b) a radiation sensitive layer. After the metal salt coating has dried, a radiation sensitive coating can be placed on the surface. The radiation sensitive coating is placed directly on the lithographic printing plate support material, or preferably, over one or more subbing layers. Various radiation sensitive materials suitable for forming images for use in the lithographic printing process can be used. Almost any radiation sensitive layer is suitable which after exposure, if necessary followed by developing and/or fixing, provides an area in imagewise distribution which may be used for printing.

Radiation sensitive materials useful in this invention are well known in the art, and include silver halide emulsions, as described in Research Disclosure, publication 17643, paragraph XXV, Dec., 1978 and references noted therein; quinone diazides (polymeric and non-polymeric), as described in U.S. patent 4,141,733 (issued February 27, 1979 to Guild) and references noted therein; light sensitive polycarbonates, as described in U.S. patent 3,511,611 (issued May 12, 1970 to Rauner et al) and references noted therein; diazonium salts, diazo resins, cinnamal-malonic acids and functional equivalents thereof and others described in U.S. patent 3,342,601 (issued September 19, 1967 to Houle et al) and references noted therein; and light sensitive polyesters, polycarbonates and polysulfonates, as described in U.S. patent 4,139,390 (issued February 13, 1979 to Rauner et al) and references noted therein.

Particularly useful radiation sensitive materials are photocrosslinkable polymers, such as polyesters, containing the photosensitive group as an integral part of the polymer backbone. For example, preferred photocrosslinkable polymers are polyesters prepared from one or more compounds represented by the following formulae: wherein R² is one or more alkyl of 1 to 6 carbon atoms, aryl of 6 to 12 carbon atoms, aralkyl of 7 to 20 carbon atoms, alkoxy of 1 to 6 carbon atoms, nitro, amino, acrylic, carboxyl, hydrogen or halo and is chosen to provide at least one condensation site; and R³ is hydroxy, alkoxy of 1 to 6 carbon atoms, halo or oxy if the compound is an acid anhydride. A preferred compound is p-phenylene diacrylic acid or a functional equivalent thereof. These and other useful compounds are described in U.S. patent 3,030,208 (issued April 17, 1962 to Schellenberg et al); U.S. patent 3,702,765 (issued November 14, 1972) to Laakso); and U.S. patent 3,622,320 (issued November 23, 1971 to Allen). R³ is as defined above, and R⁴ is alkylidene of 1 to 4 carbon atoms, aralkylidene of 7 to 16 carbon atoms, or a 5- to 6-membered heterocyclic ring. Particularly useful compounds of formula (B) are cinnamylidene- malonic acid, 2-butenylidenemalonic acid, 3-pentenylidenemalonic acid, O-nitrocinnamylidenemalonic acid, naphthyallylidenemalonic acid, 2-furfurylideneethylidenemalonic acid and functional equivalents thereof. These and other useful compounds are described in U.S. patent 3,674,745 (issued July 4, 1972 to Philipot et al). R³ is as defined above; and R⁵ is hydrogen or methyl. Particularly useful compounds of formula (C) are trans,trans-muconic acid, cis,trans-muconic acid, cis,cis-muconic acid, a,a'-cis,trans-dimethylmuconic acid, a,a'-cis,cis-dimethylmuconic acid and functional equivalents thereof. These and other useful compounds are described in U.S. patent 3,615,434 (issued October 26, 1971 to McConkey). R³ is as defined above; and Z represents the atoms necessary to form an unsaturated, bridged or unbridged carbocyclic nucleus of 6 or 7 carbon atoms. Such nucleus can be substituted or unsubstituted. Particularly useful compounds of formula (D) are 4-cyclohexene-1,2.dicarboxylic acid, 5-norbornene-2,3-dicarboxylic acid, hexachloro-5[2:2:1]-bicycloheptene-2,3-dicarboxylic acid and functional equivalents thereof. These and other useful compounds are described in Canadian patent 824,096 (issued September 30, 1969 to Mench et al). R³ is as defined above; and R⁶ is hydrogen, alkyl of 1 to 12 carbon atoms, cycloalkyl of 5 to 12 carbon atoms or aryl of 6 to 12 carbon atoms. R⁶ can be substituted, where possible, with such substituents as do not interfere with the condensation reaction, such as halo, nitro, aryl, alkoxy, aryloxy, etc. The carbonyl groups are attached to the cyclohexadiene nucleus meta or para to each other, and preferably para. Particularly useful compounds of formula (E) are 1,3-cyclohexadiene-1,4-dicarboxylic acid, 1,3-cyclohexadiene-1,3-dicarboxylic acid, 1,3-cyclohexadiene-1,3-dicarboxylic acid, 1,5-cyclohexadiene-1,4-dicarboxylic acid and functional equivalents thereof. These and other useful compounds are described in Belgian patent 754,892 (issued October 15, 1970).

The radiation-sensitive coating can be prepared by dispersing the radiation sensitive composition or polymer in any suitable solvent or combination of solvents used in the art.

Radiation-sensitivity can be stimulated in the coating composition by incorporating therein a sensitizer. Suitable sensitizers include anthrones, such as 1-carbethoxy-2-keto-3-methyl-2- azabenzanthrone, benzanthrone; nitro sensitizers; triphenylmethanes; quinones; cyanine dye sensitizers; naphthone sensitizers such as 6-methoxybeta-2-furyl-2-acrylonaphthrone; pyrylium or thiapyrylium salts, such as 2,6-bis(p-ethoxyphenyl)-4-(p-n-amyloxyphenyl)-thiapyrylium perchlorate and 1,3,5-triphenyl- pyrylium fluoroborate; furanone; 4-picoline-N-oxide; anthraquinones such as 2-chloroanthraquinone; thiazoles such as 2-benzoylcarbethoxymethylene-1-methyl-betanaphthothiazole and methyl-2-(n-methyl- benzothiazolylidene) dithioacetate; methyl 3-methyl-2-benzothiazolidene dithioacetate; thiazolines such as 3-ethy)-2-benzoy)methy)enenapho[1,2-d]-thiazo)ine, benzothiazoline, (2-benzoylmethylene)-1-methyl-beta- naphthothiazoline; 1,2-dihydro-1-ethyi-2-phenacyiidenenaphtho[1,2-d]-thiazoie; and naphthothiazoline; quinolizones, Michler's ketone; and Michler's thioketone.

In addition to the sensitizers, a number of other addenda can be present in the coating composition and ultimately form a part of the lithographic plate. For example, dyes or pigments may be included to obtain colored images to aid in recognition. Other components which can be advantageously included in the coating composition are materials which serve to improve film formation, coating properties, adhesion of the coatings to the support, mechanical strength and stability.

The lithographic printing plate of the present invention can be exposed by conventional methods, for example through a transparency or a stencil, to an imagewise pattern of actinic radiation. Suitable radiation sources include carbon arc lamps, mercury vapor lamps, fluorescent lamps, tungsten filament lamps, photoflood lamps, lasers and the like.

The exposed lithographic printing plate can be developed using conventional developer and developing techniques. For example, in developing the lithographic printing plates incorporating radiation-sensitive polysters noted above, the developer composition is applied to the surface of the plate for a period of time sufficient to remove the polymer from non-image areas of the plate. Gentle mechanical action aids in removing the polymer composition from these areas. Thus, swabbing is a useful method of applying the developer composition to the plate. The developer composition is typically used at room temperature but it can be employed at elevated temperatures up to about 32°C. After the initial application of the developer composition, a second application can be applied, followed by either a single or double application of a desensitizing composition. The plate is then dried.

The following examples further illustrate the invention:
Example 1 and Comparative Examples A-B

An aluminum plate was immersed in a caustic solution to remove oil and dirt from the surface. The surface was grained with a brush and a slurry of abrasive media. Loose residue was removed by etching in a caustic solution followed by a nitric acid desmutting bath. The aluminum plate was anodized in a phosphoric acid electrolyte.

The plate of Comparative Example A was coated with a thin layer of polyacrylamide at a coverage of 14 mg/m². The plate was coated with a radiation sensitive coating as described in U.S. 3,030,308, a condensation of hydroxy ethoxy cyclohexane and p-phenylenediethoxy acrylate.

The plate of Comparative Example B was prepared and anodized as described above. The anodized support was treated in a 2% solution of PQ-D sodium silicate sold by PQ Corporation. The SiO₂ to Na₂0 ratio was 2:1. The support was immersed in a bath having a temperature of 82°C for 45 seconds. The support was rinsed, dried and coated with a polyacrylamide and a radiation sensitive layer as described above.

The plate of Example 1 was prepared and anodized as described above and treated in a 2% solution of PQ-D sodium silicate in a 86°C bath for 30 seconds. The plate was immersed in an aqueous bath containing 2% zinc acetate for 30 seconds. The bath temperature was 65°C. The support was rinsed, dried and coated with a polyacrylamide and a radiation sensitive layer as described above.

The dried plates were contacted to a film original including a step tablet having 14 gradations and exposed to a radiation source rich in UV radiation. The exposed plates were processed with a negative developer, treated with a lithographic plate finisher and dried. The developer and finisher are described in Examples 1-8 of U.S. patent 4,419,437.

The press sensitivity and shelf-life of the plates were determined as follows: The shelf-life of the plates was determined by measuring the Log E speed shift of the coated plate using the step tablet after a 2-week incubation period at 49°C as compared to the speed of a fresh non-incubated plate. The press sensitivity test measures the rate at which a plate sheds ink from the non-image areas and involves mounting the plate on a printing press. The press is started such that the plate receives an overall ink charge to both the image and non-image areas, i.e., the dampening system is not applied. The dampening system thereafter is applied, and prints are made as the ink sheds from the non-image areas. This procedure is repeated for ten 5-minute holds. The results are calculated from a final one-hour eleventh hold and are determined from background ink density measurements taken from the first twenty sheets. The results are reported as a comparison to the performance of commercially available Kodak Polymati6Tm Litho Plates.

Comparative Example B demonstrated a dramatic improvement in press sensitivity as compared to the unsiliciated plate of Comparative Example A. The non-exposed radiation sensitive layer of Comparative Example B, however, could not be removed by the developer indicating insolubilization of the layer due to a reaction with the silicate present on the support, rendering the plate unusable.

Example 1 of this invention indicates that a plate subjected to the treatment of this invention exhibits improved press sensitivity and excellent plate stability.

### Examples 2-3

### Effect of Bath Temperature

Plates were prepared and tested as in Example 1, except that the temperature of the zinc acetate bath was as follows:

The results indicate improving stability as the bath temperature is raised.

### Examples 4-8

### Effect of Bath Concentration

Plates were prepared and tested as in Example 1, except that the plates were immersed for 25 seconds in a 49°C bath and the concentration of the zinc acetate bath was varied as follows.

The results indicate that incubation stability reaches a maximum at a bath concentration of about 2%.

### Examples 9-16

### Effect of Bath Component

Plates were prepared and tested as in Example 1 except that the following bath components were evaluated at the following concentrations, bath temperatures and plate dwell times.

The non-exposed radiation sensitive layer of Examples 10 and 11 could not be removed by the developer. The results indicate that zinc chloride requires a higher bath temperature than does zinc acetate to effect stabilization, and that zinc acetate is the preferred salt in view of its excellent performance as an agent which improves plate stability.

### Example 17

### Effect of Radiation Sensitive Layer

A plate was prepared as described in Example 1, except that the radiation sensitive composition was a positive working copolymer of alkyl acrylate, acryloyloxyalkyl quinone diazide acid ester and acryloyloxyalkyl carboxylate repeating units, as described in U.S. 3,859,099. The silicated plate was contacted with a 3.0% zinc acetate bath at 60°C for 28 seconds. The plate of this Example was suitably exposed and processed using a suitable lithographic developer and finisher. An acceptable printing plate was provided by this process.

A plate prepared in accordance with this Example but not silicated was not acceptable. A silicated plate prepared in accordance with this Example but not subjected to a zinc acetate treatment was unusable under some handling conditions.

### Example 18

### Effect of Anodizing Electrolyte

An aluminum plate supplied by Anocoil Corporation was wire brush grained and anodized in a sulfuric acid electrolyte. A diazo resin sold by Western as Western Wipe-on resin was coated on the anodized plate to provide 75 mg/m² resin coverage. The solution was coated out of water. Olin 10G surfactant was used as a coating aid. The resulting plate was exposed to a metal halide light source through a step tablet having 14 gradations. The exposed plate was processed using tap water. To provide a visible image, the plate was handed inked with rub-up ink, rinsed and dried. The plate gained speed after incubation indicating instability.

An aluminum plate anodized as described above was silicated by immersion in a solution of sodium silicate as in Comparative Example B. The plate was coated, exposed and processed as described in this Example above. This plate was not processable after incubation, indicating very poor stability of the diazo resin coating.

An Anocoil aluminum plate was prepared as described above, except the silicating step was followed by treatment in a zinc acetate solution as in Example 1. This plate processed cleanly before and after incubation with only a slight speed gain after incubation, indicating a very stable plate.

## Claims

1. A lithographic printing plate support material comprising an anodized aluminum plate having an aniodic layer, a silicate layer in contact with the anodic layer, and a metal salt layer in contact with the silicate layer, characterized in that said metal salt layer is formed by treating the silicate layer with an aqueous bath consisting essentially of a solution of a metal salt having the formula MX wherein M is a metal selected from the group consisting of zinc, magnesium, nickel, and chromium and X is an anion selected from the group consisting of acetate, chloride and borate.

2. The lithographic support material of claim 1 wherein said metal salt is zinc acetate.

3. A lithographic printing plate comprising a radiation-sensitive layer and the support of claim 1 or claim 2.

4. The plate of claim 3 further comprising a hydrophilic layer.

5. A method of preparing a lithographic printing plate support material comprising the steps of
a) treating an anodized aluminum plate with an aqueous solution of silicating agent, the silicating agent being present at a concentration of from 0.5 to 10% and the temperature of the solution being between 20 to 100°C;
b) immersing the silicated plate in an aqueous bath consisting essentially of a metal salt having the formula MX wherein M is a metal selected from the group consisting of zinc, magnesium, nickel, and chromium, and X is an anion selected from the group consisting of acetate, chloride and borate, said metal salt being present at a concentration of from 1 to 10% at a temperature between 30 to 80°C.

6. The method of claim 5 wherein the metal salt is Zn acetate present at a concentration of from 2 to 5% and the temperature of the metal salt bath is between 50 to 70°C.

## Patentansprüche

1. Lithographisches Druckplattenträgermaterial mit einer anodisierten Aluminiumplatte und einer anodischen Schicht, einer Silikatschicht in Kontakt mit der anodischen Schicht und einer Metallsalzschicht in Kontakt mit der Silikatschicht, dadurch gekennzeichnet, daß die Metallselzschicht durch Behandlung der Silikatschicht mit einem wäßrigen Bad erzegt worden ist, das im wesentlichen aus einer Lösung eines Metallsalzes der Formel MX besteht, in der M für ein Metall, ausgewählt aus der Gruppe bestehend aus Zink, Magnesium, Nickel und Chrom und X für ein Anion, ausgewählt aus der Gruppe bestehend aus Acetat, Chlorid und Borat stehen.

2. Lithographisches Trägermaterial nach Anspruch 1, in dem das Metallsalz aus Zinkacetat besteht.

3. Lithographische Druckplatte mit einer strahlngsempfindlichen Schicht und dem Träger gemäß Anspruch 1 oder Anspruch 2.

4. Platte nach Anspruch 3, die ferner eine hydrophile Schicht aufweist.

5. Verfahren zur herstellung eines lithographischen Druckplattenträgermaterials mit den Stufen
a) Behandlung einer anodisierten Aluminiumplatte mit einer wäßrigen Lösung eines silikatisierenden Mittels, wobei das silikatisierende Mittel in einer Konzentration von 0,5 bis 10% vorliegt und die Temperatur der Lösung zwischen 20 und 100°C liegt;
b) Eintauchen der silikatisierten Platte in ein wäßriges Bad, das im wesentichen ein Metallsalz der Formel MX enthält, in der M für ein Metall, ausgewählt aus der Gruppe bestehend aus Zink, Magensium, Nickel und Chrom steht und X ein Anion, ausgewählt aus der Gruppe bestehend aus Acetat, Chlorid, und Borat ist, wobei das Metallsalz in einer Konzentration von 1 bis 10% vorliegt, bei einer Temperatur zwischen 30 und 80°C.

6. Verfahren nach Anspruch 5, in dem das Metallsalz Zn-Acetat ist, das in einer Konzentration von 2 bis 5% vorliegt und bei dem die Temperatur des Metallsalzbades zwischen 50 und 70°C liegt.

## Revendications

1. Matériau de support de plaque d'impression lithographique comprenant une plaque d'aluminium anodisé ayant une couche formée par anodisation, une couche de silicate en contact avec la couche formée par anodisation, et une couche de sel métallique en contact avec la couche de silicate, caractérisé en ce que ladite couche de sel métallique est formée en traitant la couche de silicate avec un bain aqueux consistant essentiellement en une solution de sel métallique ayant la formule MX oü M est un métal choisi parmi le zinc, le magnésium, le nickel et le chrome et X est un anion choisi parmi les ions acétate, chlorure et borate.

2. Matériau de support lithographique selon la revendication 1 dans lequel le sel métallique est l'acétate de zinc.

3. Plaque d'impression lithographique comprenant une couche sensible au rayonnement et le support de la revendication 1 ou de la revendication 2.

4. Plaque selon la revendication 3 comprenant de plus une couche hydrophile.

5. Procédé de préparation d'un matériau de support de plaque d'impression lithographique comprenant les étapes suivantes:
a) on traite une plaque d'aluminium anodisé avec une solution aqueuse d'agent silicatant, l'agent silicatant étant présent à une concentration comprise entre 0,5 et 10% et la température de la solution étant comprise entre 20 et 100°C;
b) on immerge la plaque silicatée dans un bain aqueux comprenant essentiellement un sel métallique ayant la formule MX où M est un métal choisi parmi le zinc, le magnésium, le nickel et le chrome et X est un anion choisi parmi les ions acétate, chlorure et borate, ledit sel métallique étuant présent à une concentration comprise entre 1 et 10% à une température comprise entre 30 et 80°C.

6. Procédé selon la revendication 5 dans lequel le sel métallique est l'acétate de zinc présent à une concentration comprise entre 2 et 5% et la température du bain de sel métallique est comprise entre 50 et 70°C.
